# EUROPEAN PATENT SPECIFICATION

(11) **EP 2 607 513 B1**
(45) Date of publication and mention of the grant of the patent: **06.04.2016**
(21) Application number: 12194924.2
(22) Date of filing: 29.11.2012
(51) Int. Cl.: C22C 38/00

(54) **Shape memory stainless steels with rare earth elements Ce and La**
Formgedächtnisedelstahl mit den Seltenerdelementen Ce und La
Aciers inoxydables à mémoire de forme avec des éléments de terre rares Ce et La

(30) Priority: 22.12.2011 IN CH45252011
(43) Date of publication of application: 26.06.2013
(73) Proprietor: Airbus Engineering Centre India, 560048 Bangalore (IN)
(72) Inventor: SHETTY, Kishora, 560048 BANGALORE (IN)
(74) Representative: Ribeiro, James Michael

(56) References cited:
- DE-A1- 2 447 137
- DE-B- 1 024 719
- JP-A- 4 154 909

## Description

### FIELD OF TECHNOLOGY

The present subject matter relates to shape memory stainless steels. More particularly, the present subject matter relates to shape memory stainless steels with rare earth elements Cerium (Ce) and Lanthanum (La).

### BACKGROUND

Shape memory alloys are a promising class of advanced materials used in many high technology applications, such as aerospace, electronics, and biotechnology. The shape memory alloys at a high temperature can be used as functional materials, such as actuators for aircraft engines, automobiles and pipe couplings. Further, the shape memory alloys are used to absorb wind energy. Typically, Nickel-Titanium (Ni-Ti) and Copper (Cu) based shape memory alloys have been used in such high technology applications. Even though the Nickel-Titanium (Ni-Ti) and Copper (Cu) based shape memory alloys have good shape memory effect, however their mechanical properties are lower and are significantly more expensive to produce when compared with shape memory stainless steels. Further, machinability of the Ni-Ti based shape memory alloys is relatively poor when compared with the shape memory stainless steels.

Generally, the shape memory stainless steels are cheaper alternatives to the expensive Ni-Ti and Cu based shape memory alloys. The existing shape memory stainless steels exhibit good shape memory effect, mechanical properties, machinability, weldability and corrosion resistance. However, the shape memory effect of the shape memory stainless steels is not as good as the Ni-Ti and Cu based shape memory alloys. DE1024719 discloses a thermoformable steel alloy including a "mixed metal" combination of Ce and La.

It is well known that the shape memory effect in Iron (Fe) based shape memory alloys is associated with the transformation of face centred cubic austenite (γ) to hexagonal closed packed (hcp) ε - martensite. The transformation can be divided into two components, such as one involving formation of ε - martensite when cooled below a martensite start temperature (Ms) and the other involving stress induced transformation of austenite. There are different opinions on the effect of thermal martensite on recovery strain of the Fe based shape memory alloys. One technique that is used to reduce an incidence of thermal martensite is to reduce Ms by decreasing the austenite grain size, such as addition of grain refining elements, thermo-mechanical treatments and so on.

SUMMARY Shape memory stainless steels with rare earth elements Cerium (Ce) and Lanthanum (La) are disclosed. According to one aspect of the present subject matter, the shape memory stainless steels with rare earth elements include Manganese (Mn), Silicon (Si), Chromium (Cr), Nickel (Ni), Carbon (C), Ce, La and Iron (Fe). The shape memory stainless steels with rare earth elements Ce and La include, by weight, about 15 to 17% of Mn, about 5 to 6% of Si, about 9 to 12% of Cr, about 8 to 10% of Ni, about 0.03 to 0.06% of C, about 0.10 to 0.50% of Ce, about 0.5 to 1.0% of La, unavoidable impurities, and the balance being Fe.

According to another aspect of the present subject matter, raw materials including Mn, Si, Cr, Ni, C, Ce, La and Fe in the proportions given above are melted to form a molten alloy of the shape memory stainless steels with rare earth elements Ce and La. Further, the molten alloy is solidified to form an ingot. Furthermore, the ingot is subjected to nondestructive evaluation to assess internal soundness of the ingot. In addition, the evaluated ingot is homogenized to form homogenized shape memory stainless steels with rare earth elements Ce and La. Moreover, a semi-finished product is formed from the homogenized shape memory stainless steels with rare earth elements Ce and La. Also, a desired component is formed from the semi-finished product.

The method disclosed herein may be implemented in any means for achieving various aspects. Other features will be apparent from the accompanying drawings and from the detailed description that follow.

### BRIEF DESCRIPTION OF THE DRAWINGS

Various embodiments are described herein with reference to the drawings, wherein:
**FIG.** 1 illustrates a flow diagram of an exemplary method of forming shape memory stainless steels with rare earth elements Cerium (Ce) and Lanthanum (La); and
FIG. 2 is a table including a range, by weight, of each element in the shape memory stainless steels with rare earth elements Ce and La, according to one embodiment.

The drawings described herein are for illustration purposes only and are not intended to limit the scope of the present disclosure in any way.

### DETAILED DESCRIPTION

Shape memory stainless steels with rare earth elements Cerium (Ce) and Lanthanum (La) are disclosed. In the following detailed description of the embodiments of the present subject matter, references are made to the accompanying drawings that form a part hereof, and in which are shown by way of illustration specific embodiments in which the present subject matter may be practiced. These embodiments are described in sufficient detail to enable those skilled in the art to practice the present subject matter, and it is to be understood that other embodiments may be utilized and that changes may be made without departing from the scope of the present subject matter. The following detailed description is, therefore, not to be taken in a limiting sense, and the scope of the present subject matter is defined by the appended claims.

FIG. 1 illustrates a flow diagram 100 of an exemplary method of forming shape memory stainless steels with rare earth elements Ce and La. At block 102, raw materials including Manganese (Mn), Silicon (Si), Chromium (Cr), Nickel (Ni), Carbon (C), Ce, La and Iron (Fe) are added. In one embodiment, as shown in **FIG.** 2, the shape memory stainless steels with rare earth elements Ce and La include, by weight, about 15 to 17% of Mn, about 5 to 6% of Si, about 9 to 12% of Cr, about 8 to 10% of Ni, about 0.03 to 0.06% of C, about 0.10 to 0.50% of Ce, about 0.5 to 1.0% of La and the balance being Fe. At block 104, the added raw materials are melted to form a molten alloy of the shape memory stainless steels with rare earth elements Ce and La. In one embodiment, the added raw materials are melted at a temperature of about 1600 °C to form the molten alloy. In this embodiment, the added raw materials are melted conventionally or using vacuum induction at the temperature of about 1600 °C to form the molten alloy.

At block 106, the molten alloy is solidified to form an ingot. In one embodiment, the molten alloy is solidified by cooling to form the ingot of a desired shape. At block 108, the ingot is subjected to nondestructive evaluation to assess internal soundness of the ingot based on quality parameters, such as internal defects, voids, cracks, cavities and the like. In one embodiment, the nondestructive evaluation uses gamma radiography. At block 110, the evaluated ingot is homogenized to form homogenized shape memory stainless steels with rare earth elements Ce and La. In one embodiment, the evaluated ingot is homogenized by heating the evaluated ingot at a temperature in a range of about 1050 °C to 1150 °C for about 6 hours to form the homogenized shape memory stainless steels with rare earth elements Ce and La. At block 112, a semi-finished product is formed from the homogenized shape memory stainless steels with rare earth elements Ce and La. Exemplary semi-finished product includes a rolled product, a forged product and the like. At block 114, a desired component is formed from the semi-finished product. In one embodiment, the semi-finished product is cold worked or machined to form the desired component. Exemplary desired component includes an actuator for an aircraft engine, an automobile component, a pipe coupling and the like.

In one embodiment, to measure shape memory effect of the shape memory stainless steels with rare earth elements Ce and La, thin sheets of the homogenized shape memory stainless steels with rare earth elements Ce and La are made and then small strips are extracted from the thin sheets. In one embodiment, strips with different lengths are extracted from the thin sheets to measure the shape memory effect. Further, the strips are bent into a semicircular shape on mandrels with different diameters at a room temperature with the ends of strips perpendicular to horizontal straight line. Furthermore, pre-strain (ε_{ρ}) is computed for each strip using an equation: ${ε}_{p} = t / d$ where t is thickness of the strips and d is diameter of the semicircular shapes of a respective strip.

The strips are then allowed to recover at a temperature in a range about 400 °C - 450 °C. In addition, a degree of shape recovery (η_{SME} ) for each strip is computed using an equation: ${η}_{SME} = \left(\left(90-θ\right)/90\right) \times 100$ where θ is a residual angle.

Also, the shape memory effect (also referred as a net reversible strain {ε_{R})), in percentage, for each strip is computed using an equation: ${ε}_{R} = {ε}_{P} \times {η}_{SME .}$

Referring now to **FIG. 2****,** a table 200 including a range, by weight, of each element in the shape memory stainless steels with rare earth elements Ce and La, according to one embodiment. In the table 200, the first row includes various elements in the shape memory stainless steels with rare earth elements Ce and La, such as Mn, Si, Cr, Ni, C, Ce, La and Fe. Further in the table 200, the second row includes the range, by weight, of each element in the shape memory stainless steels with rare earth elements Ce and La. Using the range of the elements, in the table 200, one can form multiple shape memory stainless steels with rare earth elements Ce and La.

In various embodiments, the method described in **FIGS. 1** and **2** enables to form the shape memory stainless steels with rare earth elements Ce and La. The shape memory stainless steels with rare earth elements Ce and La are cheaper compared to existing shape memory alloys. Further, the shape memory stainless steels with rare earth elements Ce and La have good mechanical properties, machinability, weldability and corrosion resistance.

## Claims

1. Shape memory stainless steels with rare earth elements Cerium (Ce) and Lanthanum (La), which comprise, by weight, 15 to 17% of Manganese (Mn), 5 to 6% of Silicon (Si), 9 to 12% of Chromium (Cr), 8 to 10% of Nickel (Ni), 0.03 to 0.06% of Carbon (C), Ce, La, unavoidable impurities, and the balance being Iron (Fe), wherein the shape memory stainless steels with rare earth elements Ce and La comprise, by weight, 0.10 to 0.50% of Ce and 0.5 to 1.0% of La.

2. A method of forming shape memory stainless steels with rare earth elements Cerium (Ce) and Lanthanum (La), comprising:
melting raw materials including, by weight, 15 to 17% of Manganese (Mn), 5 to 6% of Silicon (Si), 9 to 12% of Chromium (Cr), 8 to 10% of Nickel (Ni), 0.03 to 0.06% of Carbon (C), Ce, La and the balance being Iron (Fe) to form a molten alloy of the shape memory stainless steels with rare earth elements Ce and La, wherein the shape memory stainless steels with rare earth elements Ce and La comprise, by weight, 0.10 to 0.50% of Ce and 0.5 to 1.0% of La;
solidifying the molten alloy to form an ingot;
subjecting the ingot to nondestructive evaluation to assess internal soundness of the ingot; and
homogenizing the evaluated ingot to form homogenized shape memory stainless steels with rare earth elements Ce and La.

3. The method of claim 2, wherein homogenizing the evaluated ingot to form the homogenized shape memory stainless steels with rare earth elements Ce and La comprises:
homogenizing the evaluated ingot by heating the evaluated ingot at a temperature in a range of 1050°C to 1150°C for about 6 hours to form the homogenized shape memory stainless steels with rare earth elements Ce and La.

4. The method of claim 2, wherein the nondestructive evaluation comprises nondestructive evaluation using gamma radiography.

5. The method of claim 2, wherein melting the raw materials to form the molten alloy comprises:
adding the raw materials; and
melting the added raw materials at a temperature of about 1600°C to form the molten alloy.

6. The method of claim 5, wherein melting the added raw materials at the temperature of about 1600°C comprises:
conventional melting of the added raw materials at the temperature of about 1600°C.

7. The method of claim 5, wherein melting the added raw materials at the temperature of about 1600°C comprises:
vacuum induction melting of the added raw materials at the temperature of about 1600°C.

8. The method of claim 2, wherein solidifying the molten alloy to form the ingot comprises:
solidifying the molten alloy by cooling to form the ingot of a desired shape.

9. The method of claim 2, further comprising:
forming a semi-finished product from the homogenized shape memory stainless steels with rare earth elements Ce and La.

10. The method of claim 9, wherein the semi-finished product comprises a rolled product or a forged product.

11. The method of claim 9, further comprising:
forming a desired component from the semi-finished product.

12. The method of claim 11, wherein the desired component is an actuator for an aircraft engine, an automobile component and a pipe coupling.

## Patentansprüche

1. Formgedächtnisedelstahl mit den Seltenerdelementen Cer (Ce) und Lanthan (La), welches nach Gewicht 15 bis 17 % Mangan (Mn), 5 bis 6 % Silizium (Si), 9 bis 12 % Chrom (Cr), 8 bis 10 % Nickel (Ni), 0.03 bis 0.06 % Kohlenstoff (C), Ce, La und unvermeidliche Verunreinigungen umfasst und wobei der Rest Eisen (Fe) ist, wobei das Formgedächtnisedelstahl mit den Seltenerdelementen Ce und La nach Gewicht 0,10 bis 0,50 % an Ce und 0,5 bis 1,0 % an La umfasst.

2. Verfahren zum Bilden von Formgedächtnisedelstahl mit den Seltenerdelementen Cer (Ce) und Lanthan (La), umfassend:
Schmelzen von Rohmaterialien, enthaltend nach Gewicht 15 bis 17 % Mangan (Mn), 5 bis 6 % Silizium (Si), 9 bis 12 % Chrom (Cr), 8 bis 10 % Nickel (Ni), 0.03 bis 0.06 % Kohlenstoff (C), Ce und La, und wobei der Rest Eisen (Fe) ist, um ein halbfertiges Produkt des Formgedächtnisedelstahls mit den Seltenerdelementen Ce und La zu bilden, wobei das Formgedächtnisedelstahl mit den Seltenerdelementen Ce und La nach Gewicht 0,10 bis 0,50 % an Ce und 0,5 bis 1,0 % an La umfasst,
Verfestigen der geschmolzenen Legierung, um einen Barren zu formen,
Unterwerfen des Barrens einer nicht-destruktiven Untersuchung, um die innere Einwandfreiheit des Barrens zu beurteilen, und
Homogenisieren des beurteilten Barrens, um einen homogenisierten Formgedächtnisedelstahl mit den Seltenerdelementen Ce und La zu bilden.

3. Verfahren nach Anspruch 2, wobei das Homogenisieren des beurteilten Barrens, um den homogenisierten Formgedächtnisedelstahl mit den Seltenerdelementen Ce und La zu bilden, umfasst:
Homogenisieren des beurteilten Barrens durch etwa 6 Stunden langes Erhitzen des beurteilten Barrens bei einer Temperatur im Bereich von 1050 °C bis 1150 °C, um den homogenisierten Formgedächtnisedelstahl mit den Seltenerdelementen Ce und La zu bilden.

4. Verfahren nach Anspruch 2, wobei die nicht-destruktive Untersuchung eine nicht-destruktive Untersuchung unter Verwendung von Gammaradiographie umfasst.

5. Verfahren nach Anspruch 2, wobei das Schmelzen der Rohmaterialien, um die geschmolzene Legierung zu bilden, umfasst:
Zusammengeben der Rohmaterialien und
Schmelzen der zusammengegebenen Rohmaterialien bei einer Temperatur von etwa 1600 °C, um die geschmolzene Legierung zu bilden.

6. Verfahren nach Anspruch 5, wobei das Schmelzen der zusammengegebenen Rohmaterialien bei der Temperatur von etwa 1600 °C umfasst:
Herkömmliches Schmelzen der zusammengegebenen Rohmaterialien bei der Temperatur von etwa 1600 °C.

7. Verfahren nach Anspruch 5, wobei das Schmelzen der zusammengegebenen Rohmaterialien bei der Temperatur von etwa 1600 °C umfasst:
Vakuuminduktionsschmelzen der zusammengegebenen Rohmaterialien bei der Temperatur von etwa 1600 °C.

8. Verfahren nach Anspruch 2, wobei das Verfestigen der geschmolzenen Legierung, um den Barren zu formen, umfasst:
Verfestigen der geschmolzenen Legierung durch Abkühlen, um den Barren gewünschter Form zu bilden.

9. Verfahren nach Anspruch 2, ferner umfassend:
Formen eines halbfertigen Produkts aus dem homogenisierten Formgedächtnisedelstahl mit den Seltenerdelementen Ce und La.

10. Verfahren nach Anspruch 9, wobei das halbfertige Produkt ein gerolltes Produkt oder ein geschmiedetes Produkt umfasst.

11. Verfahren nach Anspruch 9, ferner umfassend:
Formen einer gewünschten Komponente aus dem halbfertigen Produkt.

12. Verfahren nach Anspruch 11, wobei die gewünschte Komponente ein Stellglied für ein Flugzeugtriebwerk, eine Automobilkomponente und eine Rohrkupplung ist.

## Revendications

1. Aciers inoxydables à mémoire de forme avec les éléments de terres rares cérium (Ce) et lanthane (La), qui comprennent, en poids, 15 à 17 % de manganèse (Mn), 5 à 6 % de silicium (Si), 9 à 12 % de chrome (Cr), 8 à 10 % de nickel (Ni), 0,03 à 0,06 % de carbone (C), Ce, La, des impuretés inévitables, et le reste étant du fer (Fe), dans lesquels les aciers inoxydables à mémoire de forme avec les éléments de terres rares Ce et La comprennent, en poids, 0,10 à 0,50 % de Ce et 0,5 à 1,0 % de La.

2. Procédé de formation d'aciers inoxydables à mémoire de forme avec les éléments de terres rares cérium (Ce) et lanthane (La), comprenant :
la fusion de matières premières brutes incluant, en poids, 15 à 17 % de manganèse (Mn), 5 à 6 % de silicium (Si), 9 à 12 % de chrome (Cr), 8 à 10 % de nickel (Ni), 0,03 à 0,06 % de carbone (C), Ce, La et le reste étant du fer (Fe) pour former un alliage fondu des aciers inoxydables à mémoire de forme avec les éléments de terres rares Ce et La, dans lequel les aciers inoxydables à mémoire de forme avec les éléments de terres rares Ce et La comprennent, en poids, 0,10 à 0,50 % de Ce et 0,5 à 1,0 % de La ;
la solidification de l'alliage fondu pour former un lingot ;
le fait de soumettre le lingot à une évaluation non destructive pour estimer la santé interne du lingot ; et
l'homogénéisation du lingot évalué pour former des aciers inoxydables homogénéisés à mémoire de forme avec les éléments de terres rares Ce et La.

3. Procédé selon la revendication 2, dans lequel l'homogénéisation du lingot évalué pour former les aciers inoxydables homogénéisés à mémoire de forme avec les éléments de terres rares Ce et La comprend :
l'homogénéisation du lingot évalué par chauffage du lingot évalué à une température dans une plage de 1 050 °C à 1 150 °C pendant environ 6 heures pour former les aciers inoxydables homogénéisés à mémoire de forme avec les éléments de terres rares Ce et La.

4. Procédé selon la revendication 2, dans lequel l'évaluation non destructive comprend une évaluation non destructive à l'aide de radiographie gamma.

5. Procédé selon la revendication 2, dans lequel la fusion des matières premières brutes pour former l'alliage fondu comprend :
l'ajout des matières premières brutes ; et
la fusion des matières premières brutes ajoutées à une température d'environ 1 600 °C pour former l'alliage fondu.

6. Procédé selon la revendication 5, dans lequel la fusion des matières premières brutes ajoutées à la température d'environ 1 600 °C comprend :
la fusion classique des matières premières brutes ajoutées à la température d'environ 1 600 °C.

7. Procédé selon la revendication 5, dans lequel la fusion des matières premières brutes ajoutées à la température d'environ 1 600 °C comprend :
la fusion sous vide avec chauffage par induction des matières premières brutes ajoutées à la température d'environ 1 600 °C.

8. Procédé selon la revendication 2, dans lequel la solidification de l'alliage fondu pour former le lingot comprend :
la solidification de l'alliage fondu par refroidissement pour former le lingot selon une forme souhaitée.

9. Procédé selon la revendication 2, comprenant en outre :
la formation d'un produit semi-fini à partir des aciers inoxydables homogénéisés à mémoire de forme avec les éléments de terres rares Ce et La.

10. Procédé selon la revendication 9, dans lequel le produit semi-fini comprend un produit laminé ou un produit forgé.

11. Procédé selon la revendication 9, comprenant en outre :
la formation d'un composant souhaité à partir du produit semi-fini.

12. Procédé selon la revendication 11, dans lequel le composant souhaité est un actionneur de moteur d'aéronef, un composant automobile et un raccord de tuyauterie.
